

Dec. 22, 1959

R. M. DORLAND ET AL

2,918,398

ARTIFICIAL BOARD

Filed July 6, 1955



Inventors

RODGER MALONE DORLAND  
MAXWELL MENEHIN YAN  
ELLIOTT GIBSON HESLOP

By

Bailey, Stephens and Hettig  
Attorneys

# United States Patent Office

2,918,398

Patented Dec. 22, 1959

1

2,918,398

## ARTIFICIAL BOARD

Roger Malone Dorland and Maxwell Menuhin Yan, Sault Ste. Marie, Ontario, and Elliott G. Heslop, Sturgeon Falls, Ontario, Canada, assignors, by mesne assignments, to Abitibi Corporation, Alpena, Mich., a corporation of Delaware

Application July 6, 1955, Serial No. 520,319

Claims priority, application Canada February 19, 1953

9 Claims. (Cl. 162—132)

This invention relates to a process for making artificial board and to the product of such process.

This application is a continuation-in-part of application Serial No. 362,654, filed June 18, 1953, now abandoned.

It is well known that an artificial board of the type known as hardboard can be produced by a process including the defibration and refining of fibrous material such as wood chips, followed by forming and dewatering of the wet lap on a Fourdrinier machine and consolidation under heat and pressure to provide a hard compact fibrous mass bound together by the hemicelluloses, lignins and other natural binding constituents of the wood. If desired, additional ingredients can be added, such as sizes, for example, various waxes, and additional binding materials such as synthetic resins, for example, phenol-formaldehyde resin.

A board produced in the foregoing manner has certain disadvantages in relation to modern demands. The fibers cause minute pits in the surface, thus increasing the number of coats of paint required to achieve a good paint surface. In addition, the smooth surface of the board has a dark appearance and is frequently marked with dense spots which makes it difficult to achieve a blond finish. The smooth surface of the board refers to the surface in direct contact with the flat platens of the press during final consolidation. The rough surface is imprinted with a supporting wire screen during the consolidation. For most purposes the surface appearance of this smooth surface only is of importance.

The requirement for an improved surface has become of increased importance in recent years. Rising wood costs and changing economics have made it necessary to use a higher proportion of waste wood than formerly, more of the brasher and less suitable species and even bark, and have made it essential to increase machine speeds and therefore the rate of water removal to as high a point as possible. Coarser fibers of freer drainage have been used to conform with the increased machine speeds and to offset the decrease in drainage rates produced by bark particles. Bark particles also result in a darker surface. Thus a demand for an improved surface has actually coincided with a deterioration in surface appearance.

One approach to enhancing the surface appearance of the smooth surface of the board would be to use finer fiber, and to eliminate all particles of bark from the wood chips. However, this would substantially increase the wood and refining costs. Furthermore, there is a limit to the freeness of the fiber as its freeness must not be lowered to the point where the thick hardboard mat will not form properly in the usual wet process. Such an approach is plainly unsatisfactory as being contrary to the modern trend of using more waste wood and coarser fibers.

Another solution which has previously been adopted is the overlay process in which a secondary head box is used to flow a thin layer of specially prepared fine fibers in a water suspension onto the partially formed

2

wet lap. The top layer of better fiber covers the poor fibers and bark specks and gives a board of improved appearance and surface qualities. This overlay process has serious limitations because the addition of relatively large volumes of water is necessary to make the secondary overlay stock flow and form properly. The water is difficult to remove. Special equipment is needed to provide the slush stock. Also the secondary stock tends to fill the valleys in the underlying surface and flow away from the peaks so that it is necessary to use a substantial thickness of overlay to give the desired evenness of surface. This is costly.

Yet another solution which has previously been adopted is to laminate a thin board with good surface qualities to a consolidated base sheet formed from coarser fibers. A sheet of paper can be used as the surface laminate. This procedure has the disadvantage that a large amount of adhesive is necessary to give a good bond between the base sheet and the surface sheet. Even with a large amount of adhesive the surface sheet may scale away under some conditions. Also a considerable quantity of additional equipment will be needed to make a laminate which will in fact have an even surface.

In accordance with the present invention it is proposed to apply a sheet of paper to the upper surface of the wet lap after a large proportion of the water has been removed from the wet lap but before the latter has been consolidated. It has been found that this produces an interlocking of the fibers of the paper and of the wet lap and a bonding between the paper and the wet lap due to the lignins, hemicelluloses and other natural binding constituents of the pulp. Thus there is produced a board which has the greatly improved surface qualities due to the fine fibers of the paper, in which there is an integral bonding between the paper and the underlying coarser fibers and which is of low cost as a thin surface layer is used and as little modification of the basic process is necessary.

A dry sheet of paper should be used to give increased absorbency to the binding constituents of the wet lap.

Additional strengthening of the bond between the paper and the underlying mass can be obtained by the use of a thin layer of additional binder, although this invention considered in its broadest aspect is not limited to the inclusion of such a binder. The binder tends to give a more uniform bonding by filling in and providing a bond where valleys occur in the base sheet.

Particularly good results have been obtained by using a drying oil as a binder. It has been found that, in addition to the contribution of the drying oil to the bonding of the paper sheet to the base mat, the drying oil gives surface properties comparable to those of the treated board produced by dipping or roller application of a drying oil to the surface of the board, but with the expenditure of a far smaller amount of drying oil. Part of the drying oil also gives a water resistant screen adjacent to the surface of the paper to prevent the formation of water spots which might otherwise be formed during the hot pressing step. These water spots are believed to be due to liquid water and the solubles therein being forced to the surface and the water flashing into steam on contact with the hot platen. The water soluble sugars and other substances cause discolouration. It has also been found that the oils give a pleasant translucent appearance to the surface of the board, but that in spite of this translucency dense spots on the surface of the base sheet are hidden.

The sheet of paper used as an overlay in accordance with this invention may vary widely in grade, thickness and other qualities. Preferably a low cost paper of good absorbency such as news print is used. Other suitable papers include sulphite, sulphate and neutral sulphite

semi-chemical sheets. The weight of the standard newsprint sheet which is preferred is about 11 lbs./1000 sq. ft.

The binder can be a drying oil such as linseed oil or a composition consisting of a blend of drying oils with petroleum polymers. Other drying oils in addition to linseed oil include soybean oil, tall oil and tung oil. Alternatively many other binders may be used including suitable formulations of synthetic resins such as phenolic resins, urea-formaldehyde resins and vinyl resins. Rubber latices such as butadiene-styrene latex and animal or vegetable glue or other binders also may be used. Ideally the binder should be cheap and effective in small amounts and should give a bond resistant to water, weather and heat. The binder should not stain the overlay. The quantity to be used will vary with the nature of the binder and other factors but in general a considerably lesser amount will be used than in the case of an ordinary laminate as the binder is not used as the primary bonding agent but only as an adjunct to the bonding obtained by the interlocking of fibers and use of the natural binding constituents of the base stock obtained in accordance with this invention. 1½ lbs. of solids/1000 sq. ft. of board is the recommended quantity in the case of linseed oil. The quantity used will generally be within the range of 1 to 5 lbs., but could be within the range of 0.5 to 10 lbs. The use of more than 2 lbs. does not significantly improve the adhesion of the paper to the base sheet, but more than 2 lbs. may be added to give a tougher surface. 1½ lbs. of phenolic resins and butadiene-styrene latex have also proved effective. Appropriate modifying agents, catalysts and driers may be added to the binder. Thus in the case of some drying oils, it may be desirable to add a drier such as a naphthenate of manganese, cobalt, lead or iron. In the case of linseed oil it has been found that where the oil is added prior to consolidation the heat during pressing and subsequent baking sufficiently hardens the oil.

The wet lap should be dewatered to a consistency of 60 to 75% moisture content or about  $\frac{1}{3}$  solids before the sheet of paper is applied. To reach this consistency the water is reduced first by free drainage through the wires of the Fourdrinier machine, followed by suction drainage and the application of cold pressure rolls. The wet lap emerging from the pressure rolls will have a smooth surface which facilitates the bonding of the overlay sheet of paper at this stage. In addition, most of the dewatering will have already taken place. The overlay will therefore interfere to a minimum extent with the dewatering of the pulp. The overlay sheet can be applied by rollers subsequent to the cold pressure rolling and prior to consolidation in the hot press. Where a binder is to be used it can be coated on the surface of the paper which will be in contact with the wet lap prior to the application of the paper to the wet lap. In the case of binders such as linseed oil and other drying oils it has been found that the binder can alternatively be applied to the outer surface of the paper after consolidation in the hot press. The drying out in the hot press will make the paper sufficiently absorbent for the binder to penetrate the paper overlay and the surface of the base sheet. When the board is baked the binder will form a bond between the paper and the base sheet. It is, however, preferred that the binder be applied prior to consolidation under heat and pressure since a part of the binder then forms a water resistant barrier to inhibit the formation of water spots.

In the drawings which illustrate the preferred embodiment of this invention:

Figure 1 is a diagrammatic illustration of a manner of carrying out the process of this invention.

Figure 2 is a vertical sectional view of a board produced by the process of this invention.

The preferred embodiment of this invention will be illustrated with reference to the production of  $\frac{1}{8}$ " hardboard with a newsprint overlay and using a linseed oil binder.

A furnish consisting of mixed hardwoods and softwoods in approximately equal proportions is provided by separate treatments of wood chips in defibrators A<sub>1</sub> and A<sub>2</sub> respectively and secondary refiners B<sub>1</sub> and B<sub>2</sub> and is passed into storage chests C<sub>1</sub> and C<sub>2</sub>. The wood is treated with steam prior to and during the defibrator step. The consistency of the pulp entering the storage chests is about 4½% by weight solids. The hardwood and softwood pulps are combined in approximately equal amounts in mixing chest D where the consistency is adjusted to about 3%. Here suitable sizing materials such as a wax emulsion are added. The pulp is transferred through pipe E by pump F to headbox G from whence it is fed onto the wire screen of the Fourdrinier H. At this stage the wet lap is about 3" thick. Part of the water is eliminated by free drainage in section J and further water is removed by one or more suction boxes K and one or more sets of suction rollers L. The wet lap is then passed through one or more pairs of cold pressure rollers M. Preferably several such pairs of rollers are used with a nip pressure varying from 100 lbs. per linear inch to 750 lbs. per linear inch. The wet lap sheet emerges about  $\frac{3}{4}$ " to 1" thick and with a moisture content of about 65%, and is transferred to table roller section N. At this stage the paper overlay is applied. Newsprint paper with a weight of about 11 lbs. per 1000 sq. ft. is passed from roller O between adhesive coating roller P and backing roller Q and is applied to the wet lap by roller R. The base sheet with the paper overlay is consolidated under heat and pressure in hot press S where it is subjected to pressure varying between 50 and 650 p.s.i. at temperatures of about 390° F. during a pressing cycle of about 8 minutes total cycle. From thence the board is passed to baking oven T where it is treated at 145 to 165° C. for about 3 hours or longer, after which it is humidified to about 7% moisture.

As illustrated in Figure 2 the product is a base sheet consisting of a consolidated fibrous mass U integrally bonded to overlay sheet V along line W. There is an interlocking of fibers along line W which gives a firm bond. In addition, there is the combined bonding effect of the natural binders from the pulp and the drying oil. Part of the drying oil will be adjacent to line W and will be available for bonding. Part of the drying oil will be forced outwardly by the migration of binding constituents and moisture from the wet lap to form a water resistant barrier shown as X. For the purpose of illustration barrier X is shown as being well defined. In practice it will not have clearly defined margins.

The product shown in Figure 2 has good abrasion resistance due to the drying oil, a pleasing translucent appearance and superior bending properties giving small radii bends with smooth surfaces. The fibers of the overlay are short and do not tend to pop out of the surface, and the overlay acts as a consolidating sheath for the underlying base sheet. The product should be free from dark dense spots. In addition, it has been found that about one coat of paint can be eliminated by the improved surface of the product in comparison with ordinary hardboard. As the coat of painting is several cents per square foot per coat and the cost of the impregnated overlay is only a fraction of a cent per square foot, a considerable saving is achieved. The surface effects of the product are comparable to that of board treated by immersion or roller application with between 2 and 8% of drying oil by weight of the board. It is apparent that the present process will be more economical. The present process also compares favourably with the slush overlay process in which an overlay of between 25 lbs. and 100 lbs./1000 sq. ft. of board is normally used and in which, in addition, there are higher equipment costs.

It has been found that the foregoing process can be extended to provide an improved artificial board having a surface printed with a pattern such as a simulated wood grain.

It has been found that, where a pattern is printed on the sheet of paper which is combined with the surface of the board in accordance with the process outlined above, there is excellent resistance to defacement of the pattern by abrasion as compared with post-lamination procedures in which paper having a printed surface is merely adhered to a finished board.

In an experiment conducted to confirm the foregoing, three samples were prepared, namely:

(I) A printed overlay sheet of paper combined with a  $\frac{1}{8}$ " standard base in accordance with the process described in the main disclosure using a linseed oil binder in the proportion of  $1\frac{1}{2}$  lbs. of binder to 1,000 square feet of board.

(II) A similar printed sheet of paper to (I) glued to a finished standard board using ordinary paper mucilage, cold, with slight pressure.

(III) A similar printed sheet of paper to (I) glued to a finished standard board using a latex cement, cold, with pressure to give a good bond.

Samples of each type were tested on a laboratory Taber Abraser, with the wheels of the tester being reground between each sample to provide a fresh surface each time. Observations were carefully made during each test to determine the following end points (measured in revolutions to the nearest 10) as points of comparison:

(A) The point at which the pattern lines first showed definite signs of wearing off,

(B) The point at which the pattern lines had completely disappeared,

(C) The point at which the overlay paper first showed definite signs of breaking through to the base board, and

(D) The point at which the overlay paper had completely worn off, leaving the base board showing through.

The results of these tests were as follows:

| TYPE                                          | Sample No.   | (A)<br>Pat.<br>Start.<br>wear<br>off<br>(Revs.) | (B)<br>Pattern<br>all gone<br>(Revs.) | (C)<br>Overlay<br>start to<br>break<br>through<br>(Revs.) | (D)<br>Overlay<br>all gone<br>(Revs.) |
|-----------------------------------------------|--------------|-------------------------------------------------|---------------------------------------|-----------------------------------------------------------|---------------------------------------|
| I. Process of invention with printed overlay. | 1            | 90                                              | 180                                   | 350                                                       | 700                                   |
|                                               | 2            | 70                                              | 150                                   | 290                                                       | 500                                   |
|                                               | 3            | 90                                              | 170                                   | 300                                                       | 600                                   |
|                                               | 4            | 130                                             | 210                                   | 350                                                       | 650                                   |
| Average.....                                  |              | 95                                              | 180                                   | 320                                                       | 610                                   |
| II. Mucilage—cold glued.                      | 1            | 50                                              | 70                                    | 80                                                        | 150                                   |
|                                               | 2            | 50                                              | 60                                    | 70                                                        | 140                                   |
|                                               | 3            | 60                                              | 80                                    | 80                                                        | 150                                   |
|                                               | 4            | 50                                              | 70                                    | 60                                                        | 180                                   |
| Average.....                                  |              | 50                                              | 70                                    | 70                                                        | 150                                   |
| III. Latex—cold bonded with press.            | 1            | 60                                              | 80                                    | 200                                                       | 340                                   |
|                                               | 2            | 50                                              | 70                                    | 190                                                       | 300                                   |
|                                               | Average..... | 55                                              | 75                                    | 195                                                       | 320                                   |

It will be apparent from the results of these tests that the process of this invention imparts extremely effective resistance to defacement by abrasion to patterns printed on an overlay.

We claim:

1. A process for making hardboard comprising the steps of forming a thick wet lap consisting essentially of coarse fibrous wood pulp and containing the natural lignocellulose, partially dewatering the wet lap to a solids content of 25% to 40% by weight, applying a finished sheet of paper to the surface of said partially dewatered wet lap which comprises the smooth surface of the finished board, and consolidating the wet lap into hardboard under combined heat and pressure and simultaneously consolidating the sheet of paper therewith.

2. A process as claimed in claim 1 in which said sheet of paper is substantially dry when it is applied.

3. A process as claimed in claim 1 in which said paper prior to application thereof to said wet lap has a pattern printed thereon on the surface opposite the one which is applied to the wet lap.

4. The product produced by the process claimed in claim 1.

5. A process for making hardboard comprising the steps of forming a thick wet lap consisting essentially of coarse fibrous wood pulp and containing the natural lignocellulose, partially dewatering the wet lap to a solids content of 25% to 40% by weight, applying a finished sheet of paper to the surface of said partially dewatered wet lap which comprises the smooth surface of the finished board, applying a layer of binder to a surface of said paper, and consolidating the wet lap to which the sheet of paper and binder have been applied into hardboard under combined heat and pressure and simultaneously consolidating the sheet of paper therewith.

6. A process as claimed in claim 5 which comprises the additional step of curing the consolidated hardboard to strengthen the bond between the paper and the board.

7. A process as claimed in claim 5 in which the binder is drying oil used in a quantity of about 1 to 5 lbs. to 1,000 sq. ft. of board.

8. A process as claimed in claim 5 in which the binder is applied to the paper before the paper is applied to the wet lap, and that surface of the sheet of paper to which the binder is applied is thereafter applied to the wet lap.

9. A process as claimed in claim 8 in which said paper prior to application thereof to said wet lap has a pattern printed thereon on the surface opposite the one which is applied to the wet lap.

#### References Cited in the file of this patent

#### UNITED STATES PATENTS

|    |           |           |       |               |
|----|-----------|-----------|-------|---------------|
| 50 | 242,253   | Benton    | ----- | May 31, 1881  |
|    | 513,017   | Howard    | ----- | Jan. 16, 1894 |
|    | 695,787   | Brown     | ----- | Mar. 18, 1902 |
|    | 793,832   | Engelmann | ----- | July 4, 1905  |
|    | 1,680,896 | Marr      | ----- | Aug. 14, 1928 |
| 55 | 1,941,536 | Boehm     | ----- | Jan. 2, 1934  |
|    | 1,995,145 | Frost     | ----- | Mar. 19, 1935 |
|    | 2,077,714 | Rozema    | ----- | Apr. 20, 1937 |
|    | 2,161,655 | Ellis     | ----- | June 6, 1939  |
|    | 2,167,440 | Mason     | ----- | July 25, 1939 |
| 60 | 2,348,081 | Linzell   | ----- | May 2, 1944   |